

# UNITED STATES PATENT OFFICE.

WALTER SEEGER, OF NUEREMBERG, GERMANY.

## MANUFACTURE OF MAGNETITE ELECTRODES.

1,079,269.

Specification of Letters Patent.

Patented Nov. 18, 1913.

No Drawing.

Application filed January 26, 1912. Serial No. 673,662.

To all whom it may concern:

Be it known that I, Dr. WALTER SEEGER, a subject of the German Empire, residing at Nuremberg, in the Kingdom of Bavaria, 5 Germany, have invented certain new and useful Improvements in the Manufacture of Magnetite Electrodes; and I do hereby declare the following to be a full, clear, and exact description of the invention, such as 10 will enable others skilled in the art to which it appertains to make and use the same.

My invention relates to improvements in a process of producing magnetite electrodes having an excess of ferrous oxid for use in 15 the electrolysis of chlorids of alkalis.

As is well known in the art, when heating iron in steam magnetite, that is an iron oxid of the composition  $Fe_3O_4$ , is obtained, which can be used as an electrode in the electrolysis of chlorids of alkalis. Furthermore also such iron oxids can be used as anodes in the electrolysis of chlorids of alkalis which are obtained by the combustion of iron in a current of oxygen under conditions which cause 25 the production of an excess of ferrous oxid above the formula  $FeO + Fe_2O_3 = Fe_3O_4$ . I have discovered that iron oxid electrodes of a similar character can be obtained the composition of which shows  $FeO$  and  $Fe_2O_3$  in 30 various proportions, beginning from very much  $FeO$  + very little  $Fe_2O_3$  up to very little  $FeO$  + very much  $Fe_2O_3$ , if iron is heated in steam at a temperature of about 1000 degrees centigrade. This process is 35 remarkable in this respect, that in steam of the temperature indicated the iron is at first transformed into ferrous oxid which contains but little ferric oxid, and which is gradually transformed into an iron oxid 40 the composition of which approaches the formula  $Fe_3O_4$ . What is more remarkable is the fact, that the iron oxid which is thus obtained and which is subject to a considerable change of its form, remains sufficiently 45 coherent and homogeneous to permit its use as an electrode. The reason for this property of the iron oxids may possibly be found in the fact, that the ferrous oxid becomes soft at the temperature of nearly 1000 50 degrees centigrade and therefore is more readily sintered. This however does not explain, why the magnetic oxid of iron ( $Fe_3O_4$ ) which is obtained from the ferrous oxid or apart therefrom, and which

melts at a much higher temperature also becomes homogeneous, so that it can well be used as an electrode. 55

In the manufacture of electrodes of the character described I may start either from compact or more or less finely divided iron, 60 and add thereto substances which are adapted to render the electrodes more homogeneous. As an addition of this character silicic acid is particularly useful which combines with a part of the oxids to form silicates and cements and strengthens the compound. 65

First example: An iron tube the wall of which had a thickness of 2 millimeters, and which had an inner diameter of 8 millimeters was heated 24 hours in a current of steam at a temperature of 1050 degrees centigrade. Thereby the tube was transformed into a perfectly homogeneous tube the inner diameter of which was about 3 70 millimeters, and the outer diameter of which was also considerably increased. The tube consisted of magnetic oxid of iron ( $Fe_3O_4$ ) and an excess of about 7 percentage of ferrous oxid. When the tube was used as an 75 anode in the electrolysis of chlorids of alkalis, it separated at first splinters of iron oxids, whereupon it remained almost unaltered and showed only a slight loss in iron oxids which was practically immaterial. 80

Second example: Pure iron powder was molded together with 4 percentage of silicic acid into a tubular block, and heated in the manner described with reference to the first example. I obtained a homogeneous, non-porous tube which contained 3 percentage surplus ferrous oxid. The oxid was not in any way altered by the electrolysis and its resistance was not excessive for practical purposes, so that the old opinion that for 90 this purpose only pure magnetite can be used is proved to be erroneous. 95

As compared to the old method of manufacturing magnetite electrodes which consists in casting the same from molten magnetite in molds, my improved method is preferable in this respect, that the extremely high temperatures are avoided, and that the electrode is brought into the desired form by shaping the body of iron at the outset 100 which can be done in a most convenient way. 105

An important advantage of my process consists in the fact, that by heating the iron

a shorter or longer time and varying the temperature electrodes of any desired composition can be obtained which contain determined proportions of  $FeO$  and  $Fe_3O_4$ .

5 Instead of starting from metallic iron as a raw material, I may start from such iron oxids as are produced in the course of the process. For example, if the electrolysis of an electrode shows an undesirable excess of 10 ferrous oxid, the electrode can be transformed into an electrode which contains less ferrous oxid by again heating the same in a current of steam.

I claim herein as my invention:

The herein described process of producing magnetite electrodes which contain an excess of ferrous oxid above the theoretical amount, which consists in heating iron in the presence of steam at a temperature of about 1000 degrees centigrade.

15 In testimony whereof I have hereunto set my hand.

DR. WALTER SEEGER.

Witnesses:

FRZ. LUDWIG BRAKE,  
BRUNO MÜLLER.